

Aug. 27, 1935.

B. H. SHOEMAKER

2,012,918

STABILIZED MINERAL OIL

Filed Nov. 3, 1932

3 Sheets-Sheet 1



Fig. 1

INVENTOR  
Bernard H. Shoemaker

BY  
Bruce K. Brown  
ATTORNEY

Aug. 27, 1935.

B. H. SHOEMAKER

2,012,918

STABILIZED MINERAL OIL

Filed Nov. 3, 1932

3 Sheets-Sheet 2



Fig. 2

INVENTOR  
Bernard H. Shoemaker  
BY  
Bruce K. Brown  
ATTORNEY

Aug. 27, 1935.

B. H. SHOEMAKER

2,012,918

STABILIZED MINERAL OIL

Filed Nov. 3, 1932

3 Sheets-Sheet 3



Fig. 3

INVENTOR  
Bernard H. Shoemaker  
BY  
Bruce K. Brown  
ATTORNEY

## UNITED STATES PATENT OFFICE

2,012,918

## STABILIZED MINERAL OIL

Bernard Harvey Shoemaker, Hammond, Ind.,  
assignor to Standard Oil Company, Chicago,  
Ill., a corporation of Indiana

Application November 3, 1932, Serial No. 640,968

14 Claims.

(Cl. 87—9)

This invention relates to the stabilization of mineral oils and it pertains more particularly to a process and composition for preventing sludge and color formation in lubricating oils when used 5 under conditions conducive to deterioration.

Mineral oils, and particularly lubricating oils, when used in internal combustion engines or under conditions where the oils come in contact with hot surfaces, deteriorate and form sludge, 10 deteriorate in color, form varnish-like products that deposit on the surfaces being lubricated and the viscosity of the oil increases with use. This deterioration of mineral oils is particularly noticeable with oils used to lubricate internal combustion engines used in motor vehicles and aeroplanes. The sludge formed collects on the piston rings and causes them to stick. Also, sludge collects in the oil pumps and oil lines and greatly 15 retards the flow of oil and in some cases plugs up the oil lines and small passages.

The object of my invention is to provide a method for stabilizing mineral oils, and particularly lubricating oils, against deterioration.

Another object is to provide a method for inhibiting the sludge formation of mineral oils by adding to the oil an inhibiting catalyst.

Another object is to prevent the increase in viscosity of the oil upon continued use.

Another object is to provide a method for preventing color deterioration of the oils.

A further object is to provide a process for preventing the formation of varnish-like products in lubricating oils and the staining of the parts to be lubricated.

In internal combustion engines it is very important that the lubricating oils be stable against sludge formation. I have found that motor oils have a great tendency to sludge and deteriorate at the high operating temperatures generally encountered in internal combustion engines such as are used in automobiles and aeroplanes. At these high temperatures it is common for lubricating oils to decompose and form sludge and coke on the pistons and in the ring grooves of the pistons. 45 This results in sticking of the rings which, in turn, allows more oil to gain access to the cylinder, thereby aggravating the condition, causing excessive oil consumption and loss of compression. The curve in Figure 1 illustrates the tendency of 50 a heavy Mid-Continent lubricating oil to form sludge with increase in temperature. It will be observed that at 320° F. it required about 54 hours for 10 grams of oil to form 10 mg. of sludge, whereas at 360° F. it required only 19 hours to 55 form 10 mg. of sludge. It is very important to

note that a relatively small increase in temperature will greatly increase the rate of sludge formation. The sludge stability of the oil with reference to temperature, shown in Figure 1, was determined by heating a quantity of oil to the desired temperature and bubbling air through the sample at the rate of 10 liters per hour. At intervals, 10 gram samples were withdrawn and tested for sludge by the precipitation method described in American Society of Testing Materials Proceedings, volume 24, page 967.

Another undesirable characteristic of lubricating oils is their change of viscosity upon use. The curve shown in Figure 2 illustrates this property of mineral oils. It will be observed that the Saybolt viscosity increases greatly upon use. The results expressed by the curve in Figure 2 were obtained by maintaining a Pennsylvania oil at 340° F. and bubbling preheated air through the oil at the rate of 100 to 150 liters per hour. It is 20 apparent that when mineral oils are used at elevated temperatures in internal combustion engines, the viscosity increases upon continued use, and the oil will become so viscous that a heavy load is put upon the engine, especially when starting. This is particularly noticeable in cold 25 weather.

Another common and undesirable property of mineral oils, and particularly those lubricating oils used in contact with hot surfaces, such as 30 in internal combustion engines, is the development of color. The curve in Figure 3 shows the rate of color formation when a heavy Mid-Continent lubricating oil is heated to 340° F. while air is bubbled into the oil at the rate of 10 liters 35 per hour.

I have found that mineral oils, and particularly lubricating oils, can be stabilized against deterioration as illustrated by sludge formation, increase in viscosity upon use, staining of the 40 surfaces to be lubricated and color formation, by adding to the oil a small quantity of an alkaline metal amide such as an alkali metal or alkaline earth metal amide. The amides suitable for my invention have the following general formula:



wherein X represents an alkaline monovalent metal such as the alkali metals,  $X_1$  represents 50 a divalent alkaline metal such as the alkaline 55

- earth metals, and R and R<sub>1</sub> may represent hydrogen atoms, alkyl, aryl, and/or aralkyl groups. Examples of these amides are the alkyl and di-alkyl alkali metal amines such as diethyl sodamide, dipropyl sodamides, dimethyl sodamides, dibutyl sodamides, diethyl sodamides, dihexyl sodamides, hexyl sodamides, amyl sodamides, butyl sodamides, propyl sodamides, ethyl propyl sodamides, ethyl butyl sodamides, ethyl amyl sodamides, propyl butyl sodamides, isopropyl butyl sodamides, methyl ethyl sodamide, methyl propyl sodamides, methyl butyl sodamides, di-isopropyl sodamide, and the like; aryl alkali metal amides such as phenyl sodamide, naphthyl sodamide, phenyl methyl sodamide, phenyl ethyl sodamide, phenyl butyl sodamides, diphenyl sodamide, naphthyl methyl sodamides, benzyl sodamide, dibenzyl sodamide, also the sodamides (Na-N compounds) of other aromatic amines such as the toluidines, chloroanilines, aminophenols, benzidine, and the like may be used. It should be understood that instead of using the sodium derivatives, I may use other alkali metal or alkaline earth metal derivatives such as potassium, lithium, calcium, magnesium, barium and the like.

The stabilized oils are prepared by dissolving and/or dispersing a small amount of a metal amide therein. The preferred amounts range from 0.1 to 0.001%, the amount varying with specific materials, however, larger amounts up to 1% may be used, if desired.

The following table illustrates the results obtained when a heavy Mid-Continent lubricating oil is stabilized with an alkali metal amide. These tests were obtained by heating a quantity of oil at 340° F. and bubbling air into the oil at the rate of 10 liters per hour. At intervals, a 10 gram sample of oil is withdrawn and tested for sludge.

withdrawn and may be recycled to the colloidal mill and reused.

The following table shows that the alkaline amides such as the alkali metal amides and the alkaline earth metal amides are also particularly effective for inhibiting color formation. This table shows the color stabilizing effect of sodamide (NaNH<sub>2</sub>) when added to a heavy lubricating oil.

Table II

| Example | Amount | True color after— |           | True color of control after— |            |
|---------|--------|-------------------|-----------|------------------------------|------------|
|         |        | 55 hours          | 103 hours | 15 hours                     | 23.5 hours |
| 1       | 0.5%   | 225               | 960       | 1435                         | 2000       |

It is apparent that the amides are particularly effective for inhibiting color formation. Instead of using sodamide I may use the amides of other alkaline metals such as calcium, barium, magnesium, potassium, lithium, aluminum and other metals of equal alkalinity.

Instead of using the amides stabilizing motor oils for use in internal combustion engines or for stabilizing hydrocarbon oils at elevated temperatures, they may be used to stabilize hydrocarbon oils during storage.

The term "stabilizing" is used in my application in a generic sense to include the preserving of the oil against deterioration in any of the foregoing respects, such as sludge formation, color formation, increase in viscosity, and/or the formation of varnish-like products. The alkali amides used in my invention do not appear to function as reducing agents and their stabilizing action cannot be definitely explained by the theory upon which the action of antioxidants are explained. How-

Table I

| 45 | Example | Stabilizer                    | Percent | Sludging time in hours to form— |          | True color after— |           |
|----|---------|-------------------------------|---------|---------------------------------|----------|-------------------|-----------|
|    |         |                               |         | 10 mg.                          | 100 mg.  | 15 hrs.           | 23.5 hrs. |
|    | 1       | Control                       | —       | —                               | —        | —                 | —         |
| 50 | 2       | Dibutyl sodamide              | 0.3     | 29                              | 44       | 1435              | 2000      |
|    | 3       | Diethyl sodamide              | 0.2     | 37                              | 63       | 175               | 740       |
|    | 4       | Sodamide (NaNH <sub>2</sub> ) | 0.5     | 60                              | Over 103 | 60                | 480       |

From the above table it is apparent that the alkali amides are very effective for inhibiting sludge formation. For example, it required 37 hours for 10 mg. of sludge to form when an oil was stabilized with 0.3% of dibutyl sodamide, whereas it required only 29 hours for the unstabilized oil to form 10 mg. of sludge. Also the true color of the stabilized oil was only 175 after 15 hours, whereas the control had a color of 1435. The low molecular weight amides such as diethylsodamide and sodamide are particularly effective for preserving the oil. If larger amounts of the alkyl amides are used, greater stability can be obtained.

Instead of adding the alkali amides to the oil, these compounds may be prepared in situ by dispersing colloidal sodium in the oil and then adding ammonia or a suitable alkyl or aromatic amine. Also the amines may be passed through a colloidal mill with the sodium and oil to be stabilized. After the amines and alkali metal have had time to react, the excess sodium is

ever, it is thought that the deterioration of mineral oils is accompanied by the formation of intermediate acidic products, and the alkali derivatives of amines retard the formation of these intermediate acidic products and thereby stabilize the oil against deterioration.

While I have described my invention with reference to certain oils and compounds, the scope of my invention is not limited thereby except insofar as set forth in the claims.

I claim:

1. The process for stabilizing hydrocarbon oils against deterioration which comprises adding a small proportion of an oil soluble amide having the following general formula:

$$X_1 = \left( \begin{matrix} -R \\ N \\ -R_1 \end{matrix} \right)$$

wherein X<sub>1</sub> represents a divalent alkaline metal and R and R<sub>1</sub> represent alkyl, aryl or aralkyl groups.

2. The process for stabilizing hydrocarbon oils against deterioration which comprises adding a small proportion of an amide having the general formula:



wherein X represents an alkali metal and R and R<sub>1</sub> represent hydrogen atoms, alkyl, aryl, or aralkyl groups.

10 3. The process for stabilizing hydrocarbon mineral oils against deterioration which comprises adding a small proportion of an amide having the following general formula:



20 wherein X represents an alkali metal and R represents an alkyl group or hydrogen atom and R<sub>1</sub> represents an alkyl group.

25 4. The process for stabilizing hydrocarbon mineral oils against deterioration which comprises adding a small proportion of an amide having the following general formula:



30 wherein X represents an alkali metal, R represents a hydrogen atom and R<sub>1</sub> represents an alkyl group.

35 5. The process for stabilizing hydrocarbon mineral oils against deterioration which comprises adding a small proportion of an amide having the following general formula:



40 wherein X represents an alkali metal, R represents a hydrogen atom and R<sub>1</sub> represents an aryl group.

45 6. The process for stabilizing hydrocarbon mineral oils against deterioration which comprises adding a small proportion of an amide having the following general formula:



50 50 wherein X represents an alkali metal, R represents a hydrogen atom and R<sub>1</sub> represents an aralkyl group.

55 7. The process for stabilizing hydrocarbon mineral oils against deterioration which comprises

adding a small proportion of an amide having the following general formula:



5

wherein X represents an alkali metal, R represents an alkyl group and R<sub>1</sub> represents an aralkyl group.

8. The process for stabilizing hydrocarbon mineral oils against deterioration which comprises adding thereto a small proportion of a dialkyl alkali metal amide.

10 9. The process for stabilizing hydrocarbon mineral oils against deterioration which comprises adding thereto a small proportion of an amide selected from the group consisting of dibutyl sodamide, diethyl sodamide, dipropyl sodamide, ethyl butyl sodamide, and amyl sodamide.

15 10. A hydrocarbon lubricating oil containing a small proportion of an amide having the general formula:



15

wherein X represents an alkali metal, R and R<sub>1</sub> may represent hydrogen atoms, alkyl, aryl or aralkyl groups.

11. A hydrocarbon lubricating oil containing a small proportion of an amide having the general formula:



30

wherein X represents an alkali metal, R represents a hydrogen atom or an alkyl group, and R<sub>1</sub> represents an alkyl group.

12. A hydrocarbon lubricating oil containing a small proportion of an amide having the general formula:



35

wherein X represents an alkali metal, R represents a hydrogen atom and R<sub>1</sub> represents an aryl group.

13. A sludge resistant mineral oil comprising a viscous hydrocarbon oil and from 0.1 to 0.5% of a dialkyl alkali metal amide.

14. A sludge resistant mineral oil comprising a viscous hydrocarbon oil and from 0.1 to 0.5% of an amide selected from the group consisting of dibutyl sodamide, diethyl sodamide, and ethyl propyl sodamide.

BERNARD HARVEY SHOEMAKER.

40

45

50

55